

## UNITED STATES PATENT OFFICE

2,511,629

## BONDING OF TEXTILE YARNS TO RUBBER

Donald Entwistle, Coventry, England, assignor to  
Courtaulds Limited, London, England, a British  
company

No Drawing. Application November 18, 1948.  
Serial No. 60,841. In Great Britain December  
1, 1947

4 Claims. (Cl. 154—136)

1

This invention relates to the bonding of textile yarns to rubber, for example, the bonding of cotton or viscose rayon tire cords to rubber in the production of automobile tires.

Despite the greater strength of rayon cords in comparison with cotton cords as used in tire production, rayon cords often cannot be used in simple substitution for cotton cords owing to the lower degree of bonding obtained. In order to improve the adhesion between rayon cords and rubber, many proposals have been made to treat the rayon yarns or cords with specified adhesives. The adhesives hitherto employed have generally been of a resinous character but these are not wholly satisfactory as individual resins have limitations in certain directions; for example, in some cases the resin in or on the rayon yarns may cause difficulties in the handling of the yarns preparatory to the production of tires.

The object of the present invention is to provide an improved process for bonding textile yarns to rubber.

According to the present invention, a process for the production of a composite article comprising vulcanised rubber bonded to textile yarns includes the step of vulcanising rubber in contact with yarns which have been impregnated with a compound of a metal the sulphide of which is insoluble in water.

Suitable metals are zinc, cadmium, mercury, copper, nickel and iron, preferred compounds of these metals are the hydroxides, carbonates and acetates. The metallic compounds may be applied to the yarns, or to such yarns twisted into cords as an aqueous suspension or solution. Thus in cases where a water-soluble compound such as cadmium acetate is to be used, it is sufficient to pass the yarn through an aqueous solution of the compound to obtain the desired impregnation. If a water-insoluble compound is to be used, for example zinc hydroxide or zinc carbonate, the yarn may be impregnated with a dispersion of the compound, preferably freshly-precipitated. In an alternative procedure a water-insoluble compound may be deposited in situ in the yarns by passing the yarns first through an aqueous solution of a metal compound such as the sulphate and then through a bath of a compound such as sodium carbonate, which reacts with the water-soluble metal compound to precipitate the desired metallic compound in the yarn.

A suitable proportion of the metallic compound is from 0.1 to 5 per cent, preferably from 0.5 to 1 per cent of the weight of the yarn.

2

When salts of strong acids such as sulphuric acid, nitric acid and hydrochloric acid are employed in the process according to the invention, an improved adhesion is obtained but at the same time, the physical properties of the yarn, particularly the tensile strength, are generally adversely affected, presumably as a result of the acid condition prevailing during the vulcanisation.

It is therefore preferred to employ either a hydroxide or a metal salt of a weak acid such as carbonic acid or acetic acid since on vulcanising, according to the invention, with these compounds, little or no deterioration in the physical properties of the yarn is obtained.

The invention is particularly applicable to viscose rayon yarns but can be applied to other rayon yarns, for example, those of stretched and saponified cellulose acetate. It is also applicable to articles such as conveyor belting and V driving-belts. It is also applicable to tires and similar articles made from synthetic as well as natural rubber products, such as for example, the synthetic rubbers obtained by polymerising butadiene with other polymerisable compounds such as styrene or acrylonitrile.

The process of the invention is of particular advantage in view of the high increase in the strength of the bond; another important advantage is that it enables the yarn to be treated before it is made into cords and also simplifies the handling of the yarn.

It is believed that during the vulcanising operation in accordance with the invention, the metallic compound in the yarn is converted into the sulphide by reaction with sulphur present in the rubber.

The invention is illustrated by the following examples, in which the percentages are by weight.

40

## Example 1

Viscose rayon tire yarn was passed through a 1 per cent aqueous zinc sulphate solution, hydroextracted, passed through a 0.2 per cent aqueous sodium carbonate solution to form zinc carbonate in situ in the yarn, hydroextracted once more, dried and then used for the construction of tire cords. The dried yarn contained about 0.65 per cent of zinc carbonate.

The adhesion to rubber of these cords was found to be equal to the adhesion of a similar untreated cotton cord and twice the adhesion of a cord prepared from untreated viscose rayon when tested as follows:

A number of 10 inch lengths of each type of cord are laid lengthwise on the surface of a slab of an unvulcanised rubber composition measuring 10 inches by 3 inches by  $\frac{1}{8}$  inch and gently pressed by hand into the rubber. The composition of the rubber stock is as follows, the parts being by weight:

Smoke sheets 100 parts, zinc oxide 40 parts, sulphur 3.5 parts, pine tar 1 part, stearic acid 2 parts, antioxidant (phenyl beta-naphthylamine) 1.5 parts and accelerator (mercaptobenzothiazole) 0.5 part.

The surface with the cords therein is now covered by a sheet of regenerated cellulose while the other surface is covered with a canvas sheet which is in turn covered by a sheet of regenerated cellulose. The whole assembly is now placed in a plat- en press and vulcanised at 30 lb. per square inch steam pressure for 60 minutes. The rubber slab is removed from the press and the sheets of regen- erated cellulose stripped off giving a rubber slab having the cords buried therein with the upper surfaces flush with the surface of the rubber. The canvas backing serves to render the slab in- extensible while carrying out the adhesion tests. One end of each cord is now stripped out for about one inch and pulled in a direction along the surface of the rubber, the cord being bent back through an angle of 180° during the test. The pull required to separate the rubber and the cord is determined.

An adhesion of a similar order was obtained by using a yarn obtained by passing viscose rayon tire yarn through a dispersion of freshly-precipi- tated zinc hydroxide, hydroextracting and drying.

#### Example 2

Example 1 was repeated but with the single exception that a 1 per cent aqueous nickel sul- phate solution was used in place of the zinc sul- phate bath.

The adhesion to rubber of the cords obtained was of the same order as that obtained with the cords produced in Example 1.

#### Example 3

Example 1 was repeated but with the single exception that a 1 per cent aqueous mercuric sul- phate solution was used in place of the zinc sul- phate bath.

The adhesion to rubber of the cords obtained was of the same order as that obtained with the cords produced in Example 1.

A similar result was obtained when copper sul- phate was used in place of the zinc sulphate.

#### Example 4

Viscose rayon tire yarn was passed through a 1 per cent aqueous cadmium acetate solution, hy- droextracted, dried and used for the construction of tire cords. The cords contained approximately 1 per cent of cadmium acetate.

The adhesion to rubber of the cords obtained when tested as described in Example 1 was greater than that of the untreated yarn but was slightly inferior to the adhesion obtained with the yarns obtained in Examples 1 to 3.

What I claim is:

1. A process for the production of a composite article comprising vulcanized rubber bonded to yarns of regenerated cellulose which includes the steps of impregnating the said yarn with a com- pound chosen from the group consisting of the hydroxides, carbonates and acetates of a metal chosen from the group consisting of zinc, cad- mium, mercury and nickel, placing the impregn- ated yarns in contact with unvulcanized rubber and then vulcanizing the rubber so that the yarns are bonded to the vulcanized rubber.

2. A process as claimed in claim 1 wherein the proportion of the compound is from 0.5 to about 1.0 per cent by weight of the yarn.

3. A process for the production of a composite article comprising vulcanized rubber bonded to yarns of regenerated cellulose which includes the steps of impregnating the said yarns with an aqueous solution of a water-soluble compound of a metal chosen from the group consisting of zinc, cadmium, mercury and nickel, treating the impregnated yarns with an aqueous solution of a water-soluble carbonate whereby the carbonate of the said metal is deposited in situ in the yarns, placing the impregnated yarns in contact with unvulcanized rubber and then vulcanizing the rubber so that the yarns are bonded to the vul- canized rubber.

4. A process as claimed in claim 3 wherein the proportion of compound is from about 0.5 to about 1.0 per cent by weight of yarn.

DONALD ENTWISTLE.

#### REFERENCES CITED

The following references are of record in the file of this patent:

#### UNITED STATES PATENTS

| Number    | Name     | Date           |
|-----------|----------|----------------|
| 1,184,015 | Price    | May 23, 1916   |
| 1,723,581 | Ruderman | Aug. 6, 1929   |
| 2,054,780 | Bley     | Sept. 15, 1936 |
| 2,314,976 | Gazdik   | Mar. 30, 1943  |